

## UNITED STATES PATENT OFFICE

WALTER A. BRIDGEMAN, OF OWEGO, NEW YORK, ASSIGNOR TO THE WILBUR WHITE CHEMICAL CO., OF OWEGO, NEW YORK, A CORPORATION OF NEW YORK

## WATERPROOFING OF MATERIALS

No Drawing.

Application filed April 17, 1928. Serial No. 270,807.

This invention relates to a process for waterproofing materials, particularly textile fabrics, and to a composition for use in such a process.

5 The invention broadly comprises impregnating the material to be waterproofed, first with an emulsion of a normally solid fat in an aqueous soap solution containing an aromatic phenol, and second with an aqueous 10 solution of a salt of aluminum. The invention is also directed to the novel compositions used for the first impregnation.

The following example will illustrate one method of carrying out the present invention:

Sufficient soap is dissolved in water to give a one-half to one and one-half per cent soap solution, the percentage depending on the particular soap used, such as ordinary neutral soap chips or the sodium salts of stearic or oleic acids. To obtain the best results the 20 hydrogen ion concentration should be adjusted by about pH 7.6. This can be done, for instance, by using dilute solutions of 25 caustic soda and acetic acid.

One-half per cent of phenol or cresol is now added to the soap solution. The solution is warmed to about 40° to 50° C. and sufficient melted fat added to it in a fine 30 stream to give an emulsion with a fat content of about 6 per cent. Suitable fats for this purpose include oleo-stearine, or beef or mutton tallow.

An emulsion made by the above method, 35 using neutral soap chips and oleo-stearine, has a creamy appearance and has no odor other than that imparted by the one-half per cent of phenol.

For waterproofing cloth of any kind the 40 cloth is either dipped in the above described emulsion, the emulsion being preferably at a temperature of about 40° C., or the emulsion is applied to the cloth by brush or sponge. When the cloth is thoroughly soaked the excess emulsion is either wrung out or allowed 45 to run off, and the cloth while still wet is then dipped immediately into a 3 per cent solution of iron-free aluminum sulphate.

The second operation precipitates the fat 50 used into the fibres of the cloth, together with

the phenol and an aluminum salt of the soap used for the emulsification. Obviously the aluminum sulphate may be replaced by other water soluble salts of aluminum.

Since the emulsion used in this process contains about 6 per cent of emulsified fat and only 1/2 to 1 1/2 per cent of soap, only a very small percentage of aluminum salt is precipitated on the cloth. If large quantities of aluminum soaps are precipitated on the cloth there is a tendency for these salts to oxidize and this is undesirable in case the fabric treated has already been dyed. By using the composition of the present invention any bad effect from the oxidation of the aluminum salts of the fatty acid is reduced to a minimum by the small amount precipitated.

The presence of an aromatic phenol, such as phenol or cresol, in the above described emulsion is very important. The phenol has 70 a three-fold function.

1. The free tallow or other fat on the cloth is prevented from becoming rancid and decomposing by the germicidal action of the phenol. Inasmuch as the phenol, as well as the tallow, is impregnated into the very fibres of the cloth, the objection to the use of tallow or a similar fat is thus overcome.

2. The phenol is efficacious in protecting the cloth from mildew, for instance, when the waterproofing process is applied to canvas which might come into contact with the ground.

3. The third advantage in the use of phenol is that it has a penetrating power far in excess of that of ordinary tallow or fat, and in consequence it assists in carrying the actual waterproofing agent into the center of the fibres; in other words, it insures complete impregnation.

It will thus be seen that the present invention comprises a composition of matter for use in conjunction with a precipitant, such as aluminum sulphate, for the waterproofing of materials, particularly textile fabrics, said composition comprising an emulsion of a fat, solid at ordinary temperatures, in an aqueous soap solution containing an aromatic phenol, such as phenol and cresol, and a process of waterproofing materials, particularly textile

fabrics, which comprises successively impregnating the material with an emulsion of an ordinarily solid fat in an aqueous soap solution containing an aromatic phenol, and with 5 an aqueous solution of an aluminum salt, such as aluminum sulphate.

I claim:

- 10 1. As a new product, a composition of matter suitable for use in conjunction with aluminum sulphate for the waterproofing of textile fabrics which comprises an emulsion of a fat, solid at ordinary temperature, in an aqueous soap solution containing an aromatic phenol.
- 15 2. As a new product, a composition of matter suitable for use in conjunction with aluminum sulphate for the waterproofing of textile fabrics which comprises an emulsion of oleo-stearine in an aqueous soap solution containing phenol.
- 20 3. As a new product, a composition of matter suitable for use in conjunction with aluminum sulphate for the waterproofing of textile fabrics which comprises a six per cent emulsion of oleo-stearine in an aqueous soap solution containing from one-half to one and one-half per cent of soap and one-half per cent of phenol.

In testimony whereof, I affix my signature.

30 WALTER A. BRIDGEMAN.

35

40

45

50

55

60

65